

# UNITED STATES PATENT OFFICE.

LOUIS HIPPOLYTE BARADUC-MULLER, OF PARIS, FRANCE.

METALLURGIC PROCESS TO PRODUCE METALS OR STEELS OF ALL QUALITIES.

933,357.

Specification of Letters Patent. Patented Sept. 7, 1909.

No Drawing.

Application filed June 29, 1908. Serial No. 441,045.

To all whom it may concern:

Be it known that I, LOUIS HIPPOLYTE BARADUC-MULLER, of Paris, France, have invented a new and useful Metallurgic Process to Produce Metals or Steels of all Qualities, which invention is fully set forth in the following specification.

This invention relates to a process of purifying metals and imparting thereto special properties, and more particularly to the production of steels of all qualities.

To this end the process consists in forming in contact with the melted metal to be treated the metals or alloys which will have for effect to purify or give to the melted metal the qualities required.

For the purpose of this invention, I use small bricks or blocks formed with mixtures of metallic oxides and siloxycon or metallic oxides and silicium carbid amorphous or crystalline (carborundum) or metallic oxides and "carbo-silicium" which I add at the time required to the molten metal.

Among the mixtures suitable for the purpose of this invention, the following are given by way of example, the parts being taken by weight. For further details, reference may be had to my French Patent No. 361,950, dated Nov. 29th, 1905, and first certificate of addition No. 7216, of Jan. 23, 1907.

|    |                                         |       |
|----|-----------------------------------------|-------|
| 1. | Oxycarbide of silicium (siloxycon)      | .270  |
|    | Oxid of nickel                          | 1.225 |
| 35 | Lime                                    | .056  |
|    | Magnesia                                | .040  |
|    | Sodium carbonate                        | .106  |
|    |                                         | 1.697 |
| 40 | 2. Carborundum amorphous or crystalline | .400  |
|    | Green oxid of chromium                  | .760  |
|    | Lime                                    | .056  |
|    | Magnesia                                | .040  |
| 45 | Sodium carbonate                        | .106  |
|    |                                         | 1.362 |
| 50 | 3. Carborundum amorphous or crystalline | .400  |
|    | Manganese dioxide                       | 1.740 |
|    | Lime                                    | .056  |
|    | Magnesia                                | .040  |
|    | Sodium carbonate                        | .106  |
| 55 |                                         | 2.342 |

When these compositions are heated to an

elevated temperature such as that attained in a combustion furnace or in an electric furnace, a metal, an alloy or a silicid results, depending on the nature of the composition. 60 In the example first given, in which oxycarbide of silicium is used, a metal or alloy results, and sometimes a metallic carbid. In the examples where carbid of silicium is used, a metal, an alloy and a metallic silicid results. When it is desired to increase the yield in metallic silicid, I employ carbo-silicium  $Si_2C$ , which may replace in whole or in part the oxycarbide of silicium and carbid of silicium used in my compositions. 65 70

The bricks or blocks above referred to have a density varying from about 2.05 to 2.65 while that of the metallic bath to which they are added is much higher and ranges from 7.1 to 8.9 according to the metal present, thereby enabling them to float in baths such as of copper, bronze, cast iron, steel and the like, or on the dross, while retaining their shape and quickly attaining the temperature requisite for the siloxycon, carbid of silicium or "carbo-silicium" ( $Si_2C$ ) to react on the metallic oxides and produce the desired metal, alloy or metallic silicid. The density of each of the last-named bodies when at a high temperature is greater than 80 the brick from which it is produced, and sinks into contact with the metallic bath into which it rapidly enters especially when the bath is stirred to facilitate its dissemination. 85 In proportion as the reaction goes on, the 90 bricks wear out little by little, in a space of time relatively short. The reactions between the metallic oxides and the siloxycon or silicium carbid or carbo-silicium in the bricks effected by the heat of the bath yield nearly 95 theoretic results, enabling metals, alloys or steels to be produced of definite composition, while avoiding an extra smelting operation of the bricks to obtain the metal, alloy or silicid for the bath of metal. 100

The bricks above referred to I preferably prepare in the following manner: I grind together or separately and in fine powder the ingredients of the mixture for making the brick, and when I have to deal with a superoxid of a metal, I add a proportional quantity of carbonaceous material, such as coal in fine powder, then add in fine powder 10 to 25% of clay or preferably clay-marl melting at about  $1200^{\circ}C$ . In 110 case the ingredients are ground separately, I weigh out the proportions of each wanted,

then mix them thoroughly well dry in any suitable mixing apparatus. When the mixture is homogeneous, I add 5 to 10% of water, containing  $\frac{1}{4}$  to  $\frac{1}{2}$  of its weight, according to the case, of neutral silicate of soda at 42° Baumé. The mixture being moistened in a homogeneous manner, is granulated while fresh through a sieve having large meshes and formed in molds into 10 bricks under a pressure of about 350 kilograms per square centimeter. When the bricks are taken out of the mold, they are dried in the open air or by artificial heat. The bricks when dried are sufficiently resisting and hard to be handled and transported without breaking. To make them extremely hard, they may be baked like building bricks to a temperature of 1000° C. at the most. The bricks may be agglomerated with magnesia and magnesium chlorid in solution, or with a small quantity of cement or like material. The brioks thus worked bear very well all variations of sudden changes in temperature. The bricks thus prepared are ready to be added to the metallic bath to be treated, the composition of the brick being selected in accordance with the object in view, such as purifying cast iron or steel, or introducing into the bath a metal, alloy or silicid to give the special properties desired. I preferably add the bricks just before the metal is to be poured.

What is claimed is:—

1. A process of the character described, consisting in adding to a molten bath of

metal which is to be refined or alloyed a composition containing a compound of carbon and silicium, the oxid of a metal or metals and a flux in the form of a brick capable of floating on the bath, said ingredients reacting at the temperature of the bath to produce a product acting to refine or alloy with said bath. 40

2. A process of the character described, consisting in adding to a molten bath of metal which is to be refined or alloyed a composition containing carbid of silicium, an oxid of a metal or metals and a flux in the form of a brick capable of floating on the bath, said ingredients reacting at the temperature of the bath to produce a product acting to refine or alloy with said bath. 45

3. A process of the character described, consisting in adding to a molten bath of metal which is to be refined or alloyed a composition containing oxycarbid of silicium, an oxid of a metal or metals, and a flux in the form of a brick capable of floating on the bath, said ingredients reacting at the temperature of the bath to produce a product acting to refine or alloy with said bath. 50

In witness whereof, I have hereunto signed my name in the presence of two subscribing witnesses.

LOUIS HIPPOLYTE BARADUC-MULLER.

Witnesses:

DEAN B. MASON,  
GABRIEL BELLARD.